

Feb. 5, 1946.

**C. G. GERHOLD**

2,394,164

## NONCORROSIVE MEDIA FOR HEATING TRANSFER

Filed Sept. 30, 1944



*Inventor:*  
Clarence G. Gerhold

By: Lee J. Gary.

Attorney:

## UNITED STATES PATENT OFFICE

2,394,164

## NONCORROSIve MEDIA FOR HEATING TRANSFER

Clarence G. Gerhold, Chicago, Ill., assignor to  
 Universal Oil Products Company, Chicago, Ill.,  
 a corporation of Delaware

Application September 30, 1944, Serial No. 556,621

22 Claims. (Cl. 252—71)

This invention relates to improvements in the manufacture of fused salt mixtures and to improved methods and means for handling such mixtures to prevent corrosion of the equipment with which they are brought in contact.

Fused metal salts, particularly mixed metal halides, are well suited for use as heat conductive media because of their low melting points, low vapor pressures, extreme stabilities, high heat transfer coefficients and high heat capacity per unit volume. A great deal of difficulty has been experienced, however, in using such mixtures due to corrosion of the equipment with which they are in contact. The present invention is directed towards means of eliminating this corrosion.

The corrosion in such systems falls into the two general types, namely replacement corrosion and electrolytic corrosion.

Replacement corrosion occurs when fused metal salts are employed having cations whose position in the electromotive series is lower than that of the metal of the walls of the vessel. In these cases a substitution occurs in which the metal from the walls displaces the cations in the salt mixture lower in the electromotive series thereby effecting corrosion of the walls. For example, if one of the components of the salt mixture were cuprous chloride the salt would attack a steel vessel resulting in deposition of the copper and the substitution of iron ions in the salts in place of the copper ions. This replacement reaction may be set up as follows:



If the cations are higher in the electromotive series than the metal of the walls of the vessel, for example iron, their replacement reaction  $\text{Fe} + \text{M}^{++} \rightarrow \text{Fe}^{++} + \text{M}$  cannot proceed unless energy in the form of electromotive force is applied. The magnitude of the necessary EMF decreases with the proximity of the cations  $^{++}$  to iron in the electromotive series. This latter type of corrosion is usually spoken of as electrolytic corrosion and is the more viscous of the two types in respect to the deterioration of the walls of the chamber. It has been previously proposed to add iron salts to the salt mixtures to prevent corrosion of the vessel, the thought being that the presence of iron cations in the salt mixture would in accordance with the law of mass action suppress the tendency of the iron in the vessel walls to go into solution. However, I have discovered that the rate of corrosion of iron vessels which are contacted with fused salt mixtures is directly related to the presence of iron cations in the mix-

ture. Although the exact reason for this is not known it can probably be explained as follows: As previously stated, when using salts having metal cations higher in the electromotive series than the metals of the walls of a vessel as heat carrying media, it is necessary that some electromotive force be applied before any displacement of the metal cations of the salt mixture by the metal of the vessel walls occurs. It is also true that the potential necessary decreases as the respective positions of the metals in the electromotive series approach one another. Therefore, presence of cations which are similar to the metal of the wall provides a setup in which any slight potential would be sufficient to effect displacement and the attending corrosion. Further, with increases in the concentration of the iron cations, excessive amounts of corrosion will result as a result of the increase in current density. I have discovered that by maintaining the iron cation concentration in the fused salt mixture below about 300 to 400 parts per million and preferably below about 200 parts per million, the rate of corrosion is very low and the equipment can be used for long extended periods of operation without replacement. For example, in a case in which an iron vessel contains a bath of very pure sodium aluminum chloride mixture, that is a mixture in which the cations in the bath are all considerably higher in the electromotive series than the walls of the vessel, the flow of current can only occur by corrosion of the iron and corresponding depositions of aluminum or sodium. Since this requires a definite and fairly high potential no corrosion would be encountered in such a system until this potential were reached. Theoretically speaking, therefore, if a very pure salt were maintained no difficulties with corrosion would result. However, as a practical measure it is impossible in the ordinary operation to maintain the degree of purity necessary to avoid corrosion. In equipment of commercial size ordinarily small amounts of iron are introduced into the salt mixture by scaling or perhaps by replacement corrosion which occurs if small amounts of water are present in the system forming  $\text{HCl}$ . Since hydrogen can be replaced by iron ions small amounts of iron chloride are formed in the salt mixture. As the amount of iron ions increases due to the accumulation in the salt mixture a point is reached where a very low electromotive force will cause substantial electrolytic corrosion. In vessels of commercial size this driving potential may be set up due to temperature gradients

or due to contacts with dissimilar metal. As a result of the presence of the iron cations in the salt mixtures these low potentials obtained by temperature differences in the vessel which would ordinarily be insufficient to cause excessive electrolytic corrosion may because of the low potential now necessary effect corrosion at a substantial rate and subsequently result in failure of the vessel.

I have discovered a method for effecting continuous utilization of heat carrying media by maintaining the purity of said media at a level such that no accumulation of iron cations occurs thereby substantially preventing the previously described electrolytic corrosion.

I have found that if the salt solutions are kept in contact with a metal which is higher in the electromotive series than any of the components of the vessel walls and which preferably corresponds to the cation in the salt mixture lowest in the electromotive series, the impurities in the salt solution are removed thereby preventing the accumulation of these impurities in the salt solution and eliminating or substantially reducing any electrolytic corrosion. The metal introduced into the salt solution may be in a finely divided state such as metal powder or when desired may be in the form of a plate electrode. In the latter case it is preferable that the electrode is electrically insulated from the walls of the containing vessel to prevent the metal from going into solutions and plating on the walls of said vessel.

Salt mixtures which may be employed in the process of the present invention comprise such metal salt mixtures as potassium zinc chloride, lithium aluminum chloride, sodium aluminum chloride, mixtures of sodium aluminum chloride and potassium aluminum chloride, sodium nitrate and sodium nitrite and similar materials. The preferred salt mixtures are those comprising mixtures of the halides of the alkali metals and aluminum halides and particularly the chlorides such as sodium chloride and aluminum chloride.

In selecting the metals to be employed to replace the impurities accumulating in the salt mixture it is important that the metal chosen will not upon replacement change the composition of the salt mixture appreciably in order for the characteristics of the salt mixture, such as heat capacity, etc., to remain substantially constant throughout the operation. Further, it should be noted that in some instances alloys of metals may be used instead of a single metal to effect the removal of impurities.

In a cyclic system in which the fused metal salts are passed through a heating means and then in indirect heat exchange with materials undergoing reaction such as hydrocarbon conversion reactions, for example, dehydrogenation, catalytic cracking, catalytic reforming, catalytic aromatization, etc., the process of the present invention may be used to great advantage. The advantages will be more clearly set forth herein-after in the specification and description of a catalytic dehydrogenation process to produce butadiene utilizing a fused salt mixture as a heat carrying media.

In one embodiment my invention comprises a system for effecting heat transfer employing a fused salt mixture in indirect heat exchange with the materials to be heated, said mixture being characterized in that the cations are of metals which are higher in the electromotive series than the metal of the walls of the vessel, which comprises passing said heat carrying medium through

10 a heating zone and subsequently through a zone in which a portion of the heat contained in said medium is removed by indirect heat exchange and effecting contact of said fused salt heating medium at some point in the system with a metal corresponding to at least one of the cation constituents of said metal salt mixture and preferably with a metal corresponding to cations of the metal lowest in the electromotive series.

15 The following is a description of a diagrammatic sketch of a process for the conversion of normal butane to butadiene employing a heat carrying medium consisting of a mixture of sodium and aluminum chlorides. Although the description is limited to a butadiene process, it is not intended that the general broad scope of the invention be so limited since the invention is applicable to various processes for the conversion of organic compounds, particularly hydrocarbons 20 employing some means of transferring heat from a furnace or other heating means to a reaction zone.

25 For simplification, the diagrammatic sketch includes only elements necessary for the explanation of the invention. In the present description, a two-reactor system is employed, the catalyst in one of the reactors being utilized for the conversion operation, while the catalyst in the other reactor is simultaneously undergoing regeneration 30 by the oxidation of the carbonaceous deposits laid down upon the catalyst during a previous conversion operation. By alternately contacting the catalyst with the reactants and regenerating medium, a substantially constant over-all operation 35 is obtained.

35 Referring to the drawing, normal butane is introduced in the system through line 1 containing valve 2, commingled with recycled normal butane and butylenes obtained as hereinafter set forth, and introduced into pump 3 which discharges through line 4 containing valve 5 into heating coil 6 disposed within furnace 7 wherein the combined feed is raised to a temperature sufficient to compensate for heat losses by radiation, convection, etc. and still maintain the desired temperature in catalyst tube 12. The heated combined feed leaves furnace 7 through line 8 and is directed to line 9 containing valve 10 through line 11 into catalyst tube 12 wherein it is contacted with a catalyst capable of effecting dehydrogenation of the normal butane-butylene mixture to a substantial yield of butadiene.

40 Any suitable catalyst capable of accelerating dehydrogenation may be employed in reactor tube 12 such as, for example, the oxides of the left-hand columns of Groups V and VI of the Periodic Table supported on refractory materials such as silica, alumina, particularly an alumina 45 having the characteristics of "Activated Alumina" of commerce, magnesia, titania, etc. The preferred catalyst is one comprising chromium oxide supported on "Activated Alumina" of commerce. The temperatures employed in catalyst tube 12 may be within the range of about 950° to 1200° F. and will ordinarily be in the range of about 1000° to 1150° F. for the conversion of a butane-butylene mixture to butadiene. However, due to the endothermicity of the reaction, 50 it is necessary to provide some means of maintaining a substantially constant temperature in the reaction tube. If this is not done, a considerable temperature differential will result between the inlet temperature and outlet temperature, thereby affecting the conversion and effi-

ciency of the operation. The temperature is maintained in this system by indirect heat exchange with a solution of fused salts passed through jacket 13 in contact with the outer surface of tube 12. The molten salt is passed through line 27 containing valve 28 from salt tank 26 and is pumped by pump 29 through line 30 containing valve 31 through switch valve 32 which is so operated that it can direct the flow into the annular space between tube 12 and jacket 13 or tube 21 and jacket 22 through lines 33 or 69, respectively.

In the present description, since the catalyst in tube 12 is being employed for the endothermic dehydrogenation reaction while the catalyst in tube 21 is being regenerated, the flow of heated salt is directed through switch valve 32 through line 33 into annular space between tube 12 and jacket 13. The salt passes upwardly through the annular space in contact with the outer surface of reactor tube 12 and leaves the heating zone through line 49, through switch valve 50 which directs the flow through line 51 through heating coil 52 disposed within furnace 53 wherein the salt is raised to the desired temperature necessary to compensate for all heat losses in the system and still maintain the desired temperature in the heating jacket 13. The salt leaves furnace 53 through line 54, valve 55 and is directed into salt tank 26 wherein it is contacted with bar aluminum which reduces any iron ions present in the system because of the presence of small amounts of impurities such as HCl, and said iron is deposited as a sludge in the bottom of salt tank 26. The sludge is periodically removed from tank 26 through line 56 containing valve 57. Instead of using bars of aluminum in the salt tank, finely divided aluminum may be introduced into the circulatory system and the sludge accumulated in a trap of some sort and removed from the system by this method.

As previously stated in the butane dehydrogenation process, at least two reactors are employed with the flow of hydrocarbon and regenerating gas being alternated between the reactors to give a more continuous operation. In this description, it has been assumed that the catalyst in reactor 21 is undergoing regeneration. Since this reaction is highly exothermic, it is necessary to provide some means for removing the excess heat to prevent the temperature of the catalyst from increasing to a high level which would impair the catalyst activity. This is accomplished by passing a comparatively cool stream of fused salt in indirect heat exchange with the catalyst reactor during the regeneration operation to remove the excess heat. The system employed is substantially the same as that described previously for the addition of heat to reactor 12 with the exception that furnace 53 is replaced by cooler 62. The flow of the system is as follows: The fused salt is pumped from tank 34 through suction line 35 containing valve 36 into pump 37 which discharges through line 38, valve 39 and switch valve 32 which directs the flow through the annular space between jacket 22 and reaction tube 21. The cool salt passes upwardly through said annular space, thereby absorbing excess heat during its passage and is removed through line 70 into switch valve 50 which directs the flow through line 60, valve 61, into cooler 62 wherein its temperature is reduced sufficiently to facilitate its use as a cooling medium. The cooled salt still in liquid form is passed

through line 63 containing valve 64 into tank 34 wherein it is contacted with bar aluminum to reduce the iron cations present, thereby forming a sludge and maintaining a salt in a substantially pure state. The sludge is removed through line 58 containing valve 59.

The regenerating gas usually comprising a combustion gas containing regulated amounts of oxygen is introduced into the system through line 71 and may be directed through either lines 46 or 47 containing valves 45 and 48, respectively, depending upon which reactor tube is being regenerated. As previously stated, while the catalyst in reactor tube 21 is in the process of regeneration the flow is through line 47 containing valve 48 into line 20 through the catalyst bed in reactor 21 and the carbonaceous material from the catalyst in tube 21 removed by the passage of the regenerating gas through the catalyst bed. Ordinarily, it is necessary that the regenerating gas be heated to a temperature of about 600° to 800° F. to initiate combustion. However, to simplify the explanation of the drawing, no heating means is shown. The regenerating gases are removed from tube 21 through line 23 and directed through line 43 containing valve 44 into line 42 and may be vented to the atmosphere or may be recycled through the reactor after introduction of additional oxygen-containing gases and the excess vented to maintain a constant pressure throughout the regeneration cycle.

The products of the dehydrogenation reaction are removed through line 17 into a suitable recovery system wherein the butadiene is separated from the remaining hydrocarbons by any of the well known means such as azeotropic distillation, formation of chemical compounds, etc. and the remaining material comprising normal butane and butylenes introduced through line 65 and valve 66 into line 1 wherein it is commingled with the fresh butane charge to form the combined feed to the operation.

In the above description of the drawing, the catalyst reactors have been represented as single tubes disposed in the heating jacket. However, for commercial operation, a number of tubes in two or more banks connected by a common inlet manifold are disposed within a common heating or cooling jacket with the conversion or regeneration reaction being conducted simultaneously in all the tubes in either bank.

The following example presents a comparison of the data obtained in a circulatory salt system in which a fused salt of sodium and aluminum chloride was employed as a heat carrying medium. These data were obtained by circulating a salt mixture through stainless steel equipment for a period of 132 hours.

#### Rate of penetration

| Temp., °F. | No aluminum present | Aluminum present |
|------------|---------------------|------------------|
| 1100.....  | 0.014               | 0                |

It is obvious from the above test that the presence of aluminum (1% powdered aluminum by weight) substantially decreases the corrosion rate of the salt in the equipment. To further prove this, a life test was conducted in which a stainless steel sample was placed, using a similar circulatory system and employing sodium aluminum chloride plus 1% of aluminum dust, at a tempera-

ture of 1100-1150° F. for a period of 49 days. The following data were obtained:

| Days on test | Weight | Mean diameter | Rate of penetration |
|--------------|--------|---------------|---------------------|
|              | Grams  | Inches        | Inches/year         |
| 0            | 62.59  | 0.5003        | 0                   |
| 24           | 62.44  | 0.4999        | 0.003               |
| 25           | 62.40  | 0.4996        | 0.005               |
| 32           | 62.34  | 0.4995        | 0.004               |
| 42           | 62.20  | 0.4995        | 0.004               |
| 49           | 62.05  | 0.4993        | 0.004               |

In this table, the corrosion rates are based on the total time elapsed during the test. It will be noted from the above data that over a period of 49 days the average rate of penetration in inches per year is comparatively minor, thereby indicating that the mixture employed in this test would be completely satisfactory for a heat carrying medium in commercial operations.

I claim as my invention:

1. A heat transfer method which comprises circulating a molten metal salt mixture through a confined zone in indirect heat exchange relationship with another fluid, said salt mixture being characterized in that the cations of the salts thereof are of metals higher in the electromotive series than the metals of the walls of said confined zone, and effecting contact of the circulating molten salt mixture with a metal corresponding to one of said cations.

2. In a heat transfer process wherein a molten metal salt mixture is passed through a confined zone in indirect heat exchange relationship with another fluid, said salt mixture being characterized in that the cations of the salts thereof are of metals higher in the electromotive series than the metals of the walls of said confined zone, the method which comprises circulating said heat carrying medium through a heating zone and subsequently through a zone in which a portion of the heat contained in said medium is removed by indirect heat exchange and effecting contact of the circulating molten salt mixture with at least one metal corresponding to one of said cations.

3. In a heat transfer process wherein a molten metal salt mixture is passed through a confined zone in indirect heat exchange relationship with another fluid, said salt mixture being characterized in that the cations of the salts thereof are of metals higher in the electromotive series than the metals of the walls of said confined zone, the method which comprises circulating said heat carrying medium through a heating zone and subsequently through a zone in which a portion of the heat contained in said medium is removed by indirect heat exchange and effecting contact of the circulating molten salt mixture with a metal corresponding to the cation constituent of said mixture which is lowest in the electromotive series.

4. The method of claim 2 further characterized in that said molten metal salt mixture comprises a molten mixture of metal halides.

5. The method of claim 2 further characterized in that said molten metal salt mixture comprises a molten mixture of metal chlorides.

6. The method of claim 2, further characterized in that said molten metal salt mixture comprises a mixture of an alkali metal chloride and aluminum chloride.

7. In a heat transfer process wherein a molten sodium aluminum chloride mixture is passed

through a confined zone in indirect heat exchange relationship with another fluid, the walls of said confined zone being composed of metals lower in electromotive series than aluminum, the method which comprises circulating said molten metal salt mixture through a heating zone and subsequently through a zone in which a portion of the heat contained in said molten salt mixture is removed by indirect heat exchange and contacting the circulating molten salt mixture with aluminum.

8. In a heat transfer process wherein a molten sodium aluminum chloride mixture is passed through a confined zone in indirect heat exchange relationship with another fluid, the walls of said confined zone being composed of metals lower in electromotive series than aluminum, the method which comprises passing said molten metal salt mixture together with finely divided aluminum through a heating zone and subsequently through a zone in which a portion of the heat contained in said molten salt mixture is removed by indirect heat exchange.

9. In a heat transfer process wherein a molten

metal salt mixture is passed through a confined zone having walls composed predominantly of iron in indirect heat exchange relationship with another fluid, the molten salt mixture being characterized in that the cations of the salts thereof are metals higher in the electromotive series than iron, the method which comprises passing said heat carrying medium through a heating zone and subsequently through a zone in which a portion of the heat contained in said medium is removed by indirect heat exchange and maintaining the iron cation concentration in said molten salt mixture below about 400 parts per million by contacting said molten salt mixture with a metal corresponding to one of said cations.

10. The process of claim 8 further characterized in that said molten metal salt mixture comprises a mixture of metal chlorides.

11. In a heat transfer process wherein a molten sodium aluminum chloride mixture is passed through a confined zone having walls composed predominantly of iron in indirect heat exchange relationship with another fluid, the method which comprises passing said molten salt mixture through a heating zone and subsequently through a zone in which a portion of the heat contained in said mixture is removed by indirect heat exchange and maintaining the iron cation concentration in said molten salt mixture below about 400 parts per million by contacting said mixture with aluminum.

12. In a heat transfer process wherein a molten sodium aluminum chloride mixture is passed through a confined zone having walls composed predominantly of iron in indirect heat exchange relationship with another fluid, the method which comprises passing said molten salt mixture through a heating zone and subsequently through a zone in which a portion of the heat contained in said mixture is removed by indirect heat exchange and maintaining the iron cation concentration in said molten salt mixture below about 400 parts per million by passing finely divided aluminum through said zones in admixture with the molten salt mixture.

13. A method for preventing corrosion of the walls of a retaining zone, said walls being composed predominantly of iron and contacted with a molten metal salt mixture characterized in that the cations of the salts thereof are of metals

higher in the electromotive series than iron, which comprises maintaining the iron cation concentration in said molten salt mixture below about 400 parts by weight per million by contacting said mixture with a metal corresponding to one of said cations.

14. The method for preventing corrosion of claim 13 further characterized in that said molten metal salt mixture comprises a mixture of metal halides.

15. The method for preventing corrosion of claim 13 further characterized in that said molten metal salt mixture comprises a mixture of aluminum chloride and at least one alkali metal chloride.

16. The method for preventing corrosion of claim 13 further characterized in that said molten metal salt mixture comprises sodium aluminum chloride.

17. In a heat transfer process wherein a molten mixture of metal salts is employed as an indirect heat exchange medium, the method which comprises maintaining a source of supply of said molten mixture of metal salts, cyclically circulating molten salt mixture between said source of supply and an indirect heat exchange zone defined by walls of a metal lower in the electromotive series than the metals of said salts, whereby cations of the metal of said walls tend to accumulate in the circulating molten mixture, contacting the circulating salt mixture with a metal higher in the electromotive series than the metal of said walls to reduce said cations, and separating the thus reduced cations from the circulating molten salt mixture.

18. The method as defined in claim 17 further characterized in that said metal higher in the

electromotive series than the metal of said walls corresponds to the metal of one of said salts.

19. The method as defined in claim 17 further characterized in that said metal higher in the electromotive series than the metal of said walls corresponds to the metal of said salts which is lowest in the electromotive series.

20. A heat transfer method which comprises cyclically circulating molten sodium aluminum chloride through and between a heating zone and an indirect heat exchange zone defined by walls composed predominantly of iron, whereby iron cations tend to accumulate in the circulating molten chloride, contacting the circulating molten chloride with metallic aluminum to reduce said cations and thereby deposit iron from the molten chloride, and separating the deposited iron from the circulating molten chloride.

21. A heat transfer method which comprises cyclically circulating molten sodium aluminum chloride through and between a heating zone and an indirect heat exchange zone defined by walls composed predominantly of iron, whereby iron cations tend to accumulate in the circulating molten chloride, contacting the circulating molten chloride with metallic aluminum in a separating zone between the heating zone and the heat exchange zone to reduce said cations and thereby deposit iron in the separating zone, and withdrawing the deposited iron from the separating zone.

22. The method as defined in claim 20 further characterized in that said metallic aluminum is circulated in finely divided form through said zones in admixture with the molten sodium aluminum chloride.

CLARENCE G. GERHOLD.